

# UNITED STATES PATENT OFFICE.

CARL BETHGE, OF BERLIN, GERMANY.

## COMBUSTIBLE MIXTURE FOR PRODUCING ACTINIC LIGHT.

No. 908,837.

Specification of Letters Patent.

Patented Jan. 5, 1909.

Application filed July 30, 1908. Serial No. 446,060.

*To all whom it may concern:*

Be it known that I, CARL BETHGE, a subject of the King of Prussia, German Emperor, and resident of 18 Schlesischestrasse, Berlin, 5 Kingdom of Prussia, German Empire, have invented new and Improved Combustible Mixtures for Producing Actinic Light, of which the following is a specification.

The present invention relates to the production of improved slow burning mixtures containing magnesium or other combustible metals such as aluminum or calcium for producing while burning, a light of high actinic power.

15 In order to produce such time lights it has hitherto been usual to employ an ordinary flash light mixture together with a ballast or comparatively neutral body that is to say a suitable substance such as an alkaline earth 20 in a quantity which exceeds the chemical equivalent of the magnesium or the like. Such methods however have the disadvantage that they reduce the speed of action and also the actinic power of the light produced. 25 I have now found it possible to produce a mixture which when burned gives forth a brighter light of higher actinic powers than hitherto by mixing magnesium or its equivalent in great excess with an oxid of the rare 30 earth metals or their equivalents. As the equivalent of magnesium it is well known that aluminum, calcium, barium or strontium may be employed and as the equivalent of an oxid of the rare earth metals, salts of 35 these metals which are reducible by heat or corresponding compounds of metals which when reduced are easily combustible may be employed.

The function of the rare earth or its equivalent mentioned above is to serve as an oxygen carrier and the operations taking place during the burning of the mixture may be explained, as follows: The rare earth metal compound or its equivalent is reduced 45 by the action of the magnesium or its equivalent and the reduced metal owing to its easy combustibility is oxidized by the oxygen of the atmosphere so that further quantities of magnesium, at ever increasing temperatures, are ignited, thus the ignition propagates itself gradually through the entire

mass and causes an exceedingly bright light of very high actinic powers. The intensity of the light is still further increased by the repeated burning of the rare earth metal or 55 its equivalent, which, as is well known, produces when burned an even more intense light than magnesium.

According to the present invention the intense lighting action of the rare earths may 60 be employed without the necessity of first reducing these metals in the manner which has hitherto been proposed. Such reducing is exceedingly expensive and even when reduced the rare earth metals are difficult to 65 preserve. It has also been proposed to use nitrates of the rare earths in quantities chemically equivalent to the quantity of the magnesium but only for the purpose of producing a quick burning flash light whereas 70 the object of the present invention is to produce a light of considerable duration and also of high actinic power.

The rare earth metals may, as above described, be replaced by the alkaline earths or 75 by reducible salts of the rare earths or alkaline earths, in which case, as will be readily understood, the light has the coloring corresponding to the metal employed such as strontium and calcium. The reaction of the 80 active metal which is present in excess and the repetition of this reaction with the oxids caused by the combustion of the reduced metal may also be obtained in the case of all metal compounds in which the combustion 85 of the metal easily takes place at higher temperatures and in which the metal concerned has a lower ignition temperature than the magnesium or its equivalent.

In order to obtain an exceedingly uniform 90 intensity of light compounds of vanadium in small percentages may with advantage be added as a further oxygen carrying agent.

It has further been proposed, to employ mixtures in which the magnesium, aluminum or equivalent was present in excess, thus in the French Patent No. 357478 approximately double the chemical equivalent of magnesium or the like is mixed with sulfates and oxids. In these mixtures the 95 oxids are merely added in order to produce from the flash light mixture (the mixture of 100

the magnesium and sulfates) a time light. These mixtures contain a comparatively small excess of magnesium and burn after the nature of a flash light mixture in spite of the addition of the oxids although naturally with somewhat reduced speed. In order to prolong the period of burning to that of a slow burning light mixture a considerably greater excess of magnesium must be added. 5

10 which however would not accomplish the result required in the presence of a sulfate. If on the other hand it is desired to obtain a prolongation of the combustion by the addition of oxids in the manner set forth in the

15 French patent mentioned above such large quantities of the oxids must be added that the same no longer take part in the reaction but merely act in a mechanical manner as a ballast to produce protraction of the combustion. 20 This naturally is accompanied by a very considerable reduction in the temperature and also in the intensity of the light. Further with mixtures of the kind hitherto known it is impossible to obtain such a quiet, slow and brilliant light as that obtained by 25 the present invention.

The distinguishing feature of the present invention as compared with the known methods mentioned above consists in the

30 employment of a mixture containing magnesium in great excess, for example a minimum of three times the chemical equivalent of the oxid or reducible salt, whereby an increase of the temperature and the brilliancy of the light is caused as compared with the

35 mere mechanical protraction of the combustion of a flash light secured by the addition of an oxid. Mixtures of oxid alone with magnesium, that is to say mixtures containing

40 no flash light mixture as their basis have not hitherto been employed and such mixtures are characterized by an exceedingly quiet burning. A mixture of oxids with double the chemically equivalent quantity of

45 metal burns comparatively quickly, but a very considerable prolongation of the illumination is effected by employing mixtures with at least three times the equivalent quantity of the metal.

50 The proportions may be arranged up to 10 times the equivalent. I have given the proportions of the quantities to be used in chemical equivalents as the exact numerical ratio of the weights employed may vary and care

55 has only to be taken that the necessary excess chemically of the magnesium or its equivalent is present.

The following examples may be given of suitable compositions for the light producing

mixtures prepared according to the present 60 invention:

*Examples.*

I. 250 parts magnesium powder 150 parts cerium oxid. 65

II. 250 parts magnesium powder 150 parts cerium oxid 8 parts vanadic acid.

III. 250 parts magnesium powder 100 parts oxalate of cerium.

IV. 250 parts magnesium powder 75 parts 70 calcium hydroxid.

V. 250 parts magnesium powder 50 parts cerium oxid 50 parts calcium hydroxid.

VI. 250 parts magnesium powder 50 parts 75 oxid of manganese.

VII. 250 parts magnesium powder 50 parts cerium oxid 25 parts oxid of manganese.

2 to 3 grams of the above mixtures will burn on the average for 30 seconds; greater quantities of course will burn for longer periods. 80

What I claim is:—

1. A combustible mixture for producing actinic light of uniform intensity and relatively long duration, composed of an oxid of 85 the rare earth metals, and at least three times the chemically equivalent quantity of an easily combustible metal.

2. A combustible mixture for producing actinic light of uniform intensity and relatively long duration, composed of an oxid of 90 the rare earth metals, and at least three times the chemically equivalent quantity of magnesium.

3. A combustible mixture for producing 95 actinic light of uniform intensity and relatively long duration, composed of cerium oxid, and at least three times the chemically equivalent quantity of magnesium.

4. A combustible mixture for producing 100 actinic light of uniform intensity and relatively long duration, composed of cerium oxid, at least three times the chemically equivalent quantity of magnesium, and an oxygen bearing vanadium compound. 105

5. A combustible mixture for producing actinic light of uniform intensity and relatively long duration, composed of cerium oxid, at least three times the chemically equivalent quantity of magnesium, and a 110 small percentage of vanadic acid.

In witness whereof I have hereunto set my hand in the presence of two witnesses.

CARL BETHGE.

Witnesses:

HENRY HASPER,  
WOLDEMAR HAUPT.